

Oct. 18, 1932.

## A. ABRAMS

1,882,683

# METHOD OF DIE FORMING ARTICLES FROM SULPHURIZED PAPER BOARD

Filed June 3, 1929



## UNITED STATES PATENT OFFICE

ALLEN ABRAMS, OF WAUSAU, WISCONSIN, ASSIGNOR TO MARATHON PAPER MILLS COMPANY, OF ROTHSCHILD, WISCONSIN, A CORPORATION OF WISCONSIN

## METHOD OF DIE FORMING ARTICLES FROM SULPHURIZED PAPER BOARD

Application filed June 3, 1929. Serial No. 368,001.

This invention relates to a method of and apparatus for die forming commercial articles, such as containers, from sulphurized paper board and like material.

5 An object of this invention is to provide a method of forming shaped articles from sulphurized paper board and the like.

Another object of the invention is to provide a method of forming or drawing shaped 10 articles from sulphurized paper board and the like by means of dies.

A further object of the invention is to provide an apparatus for die forming articles from sulphurized paper board and the like.

15 The above, other and further objects of the invention will be apparent from the following description, accompanying drawing, and appended claims.

According to the invention the method consists in die drawing sulphurized paper board 20 in the presence of heat at such a temperature as not to cause the sulphur in the paper to melt substantially and come to the surface of the paper and form an uneven and rough surface, or stick to the die members.

The apparatus of the invention comprises male and female forming dies, one of which is heated for the purpose of subjecting sulphurized board and the like to heat during 30 the drawing operation, the other die taking its heat from the heated die or being also directly heated.

The accompanying drawing illustrates one embodiment of the apparatus capable of being used in practicing the method.

The views of the drawing are as follows:

Figure 1 is a sectional view taken substantially on the broken line I—I of Figure 5.

Figure 2 is a fragmentary sectional view of 40 a portion of the male die showing a thermometer inserted in the same.

Figure 3 is a fragmentary sectional view of a portion of the female die showing a thermometer inserted in the lower part of the 45 die.

Figure 4 is a top plan view of a finished article formed from sulphurized board by the method and apparatus of this invention.

Figure 5 is a sectional view taken substantially on line V—V of Figure 1.

Figure 6 is a vertical section taken on line VI—VI of Figure 4.

Figure 7 is a fragmental sectional view of a portion of the female die showing a thermometer arranged to take external temperatures of the die.

The form of apparatus illustrated in the drawing is for the purpose of explanation of the invention and the invention is not to be construed as limited to an apparatus made 60 strictly in accordance with the illustrated form of the same.

The illustrated form of the apparatus comprises a male die 1 and a female die 2 which in the present instance are shaped to form finished articles like that shown in Figures 4 and 6 of the drawing.

A female die block 3 is supported in the usual manner on the bed of a press and is flanged at 4 whereby the same may be secured 70 to the bed plate of the press.

Guide posts 5 are secured in the flange 4 of the base plate 3 and extend upwardly for guiding the male die carrying member 6 which is shown as flanged at 7 and provided 75 with apertures 8 for the guide pins 5, whereby the plate 6 may have proper movement during the drawing or forming operations.

The plates 3 and 6 may be made of any metal such as cast iron and the same are 80 faced by hardened steel. The plate or member 6 has a hardened steel ring member 9 held therein by screws 10, while the female die 2 is made as a circular wall having a lateral flange 11 through which screws 12 85 pass to fasten the same to the base plate 3.

The several parts, of course, are shaped to form the desired finished article, such as that shown in Figure 4 of the drawing.

The male die moves within the member 9 under influence of the mechanism of the press, while the male die member 6 is reciprocated in a manner well understood.

The male die 1 is provided with a plurality of axially extending apertures 13, of which 95 there are four shown in the drawing. In said apertures 13 are placed heating elements 14, which may be coiled resistance wire supplied with suitable electric current, or any other suitable heating elements. The heat 100

ing elements 14 are connected by suitable conductors 15 to a source of electrical energy for heating the same.

The male die 1 has an aperture 16 drilled therein and extending towards the center of the same for the reception of a thermometer 17, whereby the internal heat of the male die member may be observed.

The base plate 3 of the female die member 10 has an aperture 18 drilled therein for receiving a thermometer 19 for like purposes.

Another thermometer 20 may be attached by means of cement or other adherent material 21 to the outside of the female die member 3 for observing the temperature of the female die.

A stripping plate 22 is arranged within the female die and is actuated in a well-known manner for stripping the finished article from the female die.

The female die plate 3 is likewise adapted to be heated by means of elements 25 extending radially toward the center thereof and connected by means of wires 26 to a source of electrical energy.

The drawing of finished articles from sulphurized paper and the like depends on several conditions, including the control of time, temperature and moisture of the sheet. The proper combination of these factors results in successful drawing, or forming by means of dies, of sulphurized board and the like.

The several thermometers 17, 19 and 20 have been indicated respectively as X-position, Y-position and Z-position, the X-position indicating the inside temperature of the male die, the Y-position indicating the inside temperature of the female die, and the Z-position the outside temperature of the female die. It is of course possible to use more thermometers if occasion demands, and if it were believed necessary to more fully ascertain the temperatures of the various parts of the apparatus.

The preformed sulphurized board or blanks of the same to be drawn are moistened slightly, the amount of moisture running from 5 to 8 pounds per thousand square feet of paper or board. As here illustrated, a moistened circular blank, at room or other ordinary temperature, is inserted in the press and the mechanism actuated, whereupon the male die carrying member 6 and the accompanying male die 1 is caused to descend, with the member 6 stopping when the same reaches the female die and the male die 1 continuing its downward movement to form or draw the sheet into whatever is the shape of the male and the female dies. The time of drawing must necessarily be short and also the temperature involved must be such as not to melt the sulphur in the paper or board to such a degree that the same will come to the surface of the board and there crystallize, or stick to the die members. Incipient melting

of the sulphur must occur to permit satisfactory drawing of the article in the die, but the conditions of time and temperature are so controlled that undue or excessive melting of the sulphur is prevented.

It has been ascertained from a long series of experiments that articles such as shown in Figure 4 of the drawing, which is a lid for an ice-cream container, may be successfully drawn within a temperature range of from about 235° to about 275° F., as measured in the hottest parts of the dies. The most successful results have been obtained with the temperature in the hottest parts of the die running from 260 to 270° F. This temperature is sufficient to soften the sulphur to a degree to allow forming or drawing of the sheets without causing the sulphur to come to the surface and there crystallize and make an objectionable surface on the finished article.

Temperatures observed from some of these experiments at the several thermometers follow:

| Female die outside temp. Mark Z | Female die inside temp. Mark Y | Male die inside temp. Mark X |
|---------------------------------|--------------------------------|------------------------------|
| °F.<br>215                      | °F.<br>266                     | °F.<br>260                   |
| 220                             | 271                            | 265                          |
| 190                             | 241                            | 235                          |

Lids for ice-cream containers, such as illustrated in Figure 4, have been successfully made in accordance with this invention using an apparatus similar to that shown in the drawing, wherein a temperature of 200° F. was observed on bottom (female) die at mark Z with the forming operation continuing for approximately 12 seconds.

This invention is not only a forming operation but also a drawing operation. A relatively deep flange, such as the margin flange 23 of the lid (Figure 4) can be satisfactorily produced without cracking by using my method.

I am aware that many changes may be made and numerous details of construction may be varied through a wide range without departing from the principles of this invention, and I therefore do not purpose limiting the patent granted hereon otherwise than necessitated by the prior art.

I claim as my invention:

1. A method of die forming sulphurized board and the like, which comprises forming and drawing said board in dies in the presence of heat and timing the draw to permit incipient melting of the sulphur without causing the sulphur to completely fuse.

2. A method of die forming articles from sulphurized board and the like which comprises forming and drawing a moistened blank of said board in dies in the presence of heat, timing the draw and controlling the heat and moisture content to permit incipient

melting of the sulphur without drawing the sulphur to the surface of the board.

3. A method of die forming a deeply flanged cover or like article from sulphurized fiber board, which comprises subjecting a blank of sulphurized fiber board under heat and pressure to a forming and drawing action between interfitting cylindrical male and female die members, the temperature to which the sulphurized fiber board is subjected being so regulated as to cause incipient melting of the sulphur without causing excessive flow of sulphur to the surface.

4. A method of die forming articles from sulphurized board and the like, which comprises moistening the board and then forming and drawing the same between heated male and female die members, maintaining the surfaces of said die members at a temperature slightly above the melting point of sulphur, and completing said forming and drawing operation before the sulphur of said sulphurized board has completely melted.

5. A method of die forming articles from sulphurized board and the like, which comprises moistening the board and then forming and drawing the same between heated male and female die members to produce a relatively steep marginal flange on the article being formed, maintaining the surfaces of said die members at substantially the melting point of sulphur, and completing said forming and drawing operation before the sulphur of said sulphurized board has completely melted.

In testimony whereof I have hereunto subscribed my name at Rothschild, Marathon County, Wisconsin.

ALLEN ABRAMS.

40

45

50

55

60

65